

## UNITED STATES PATENT OFFICE.

HARRY A. SCHWARTZ, OF CLEVELAND, OHIO, ASSIGNOR, BY MESNE ASSIGNMENTS, TO NATIONAL MALLEABLE AND STEEL CASTINGS COMPANY, OF CLEVELAND, OHIO, A CORPORATION OF OHIO.

## RUST-RESISTANT IRON.

No Drawing.

Application filed February 24, 1922. Serial No. 538,979.

*To all whom it may concern:*

Be it known that I, HARRY A. SCHWARTZ, a citizen of the United States, residing at Cleveland, Cuyahoga County, Ohio, have 5 invented new and Improved Rust-Resistant Iron, of which the following is a specification.

My invention relates to rust resistant iron, and particularly to malleable cast iron, and 10 comprises the addition of an alloying element, which does not affect the graphitization of the casting during the malleablizing process, such as copper, nickel, or cobalt, for the purpose of improving the rust resisting 15 qualities of the iron. Additions of copper in small percentages have been found to be particularly effective in bringing about such a result.

I have found that when a small amount of 20 copper which in the final product does not exceed about .25%, preferably above .15% and as near .25% as possible, is added, a copper-iron alloy is formed which has a much greater resistance to rusting than the 25 iron constituent by itself. I believe from experiment that the limit of solubility of copper in iron is about .25%, and that if copper substantially in excess of this limit is present the excess remains in the casting 30 in what appear to be unabsorbed minute particles, which contain a high percentage of copper, and these minute particles set up an electrolytic action with the iron which results in a more rapid rusting than would 35 be the case if no copper whatever is added.

In the resulting product, when malleablized, carbon, manganese, silicon, etc., appear in the usual percentages, and, so far as I have been able to ascertain, these substances have no effect upon the copper and 40 the copper has no effect upon them.

It is my experience that in malleable cast iron containing from 2.25% or higher of carbon very greatly improved rust resisting 45 qualities are obtained without affecting the other desirable qualities of the iron. For instance, in malleable cast iron of such a

composition I have found that the rusting proceeds about two-thirds to one-seventh as fast as in ordinary malleable cast iron, depending upon the conditions to which the iron is submitted. It is obvious that my invention is of particular value in connection with stove castings; radiator connections, including nipples; pipe fittings; and other 55 uses in which rust resisting qualities are desirable.

The terms and expressions which I have employed are used as terms of description and not of limitation, and I have no intention, in the use of such terms and expressions, of excluding any equivalents of the features shown or described, or portions thereof, but recognize that various modifications are possible within the scope of the 65 invention claimed.

What I claim is:

1. A highly rust resistant malleable iron casting containing approximately between .15 and .25% of copper and forming with 70 the iron a copper-iron alloy, and having such percentages of carbon, manganese, silicon and the like as are usually present in malleable cast iron.

2. A highly rust resistant malleable iron casting having therein an amount of copper up to, but not substantially exceeding, the limit of the solubility of copper in iron, said casting containing also carbon, manganese, silicon and like elements in the percentages normally found in malleable cast iron.

3. A radiator nipple comprising a highly rust resistant malleable iron casting containing copper in an amount up to, but not 85 substantially exceeding, its limit of solubility in iron and being without effect on the graphitization of the casting during malleablizing, the casting containing also such percentages of carbon, manganese, silicon 90 and like elements as are normally found in malleable cast iron.

HARRY A. SCHWARTZ.